

## 1

3,598,663

ALUMINUM ALLOY HEAT-TREATING  
Herbert Greenewald, Jr., Columbus, Ohio, assignor to  
North American Rockwell Corporation  
No Drawing. Original application Mar. 13, 1968, Ser. No.  
712,674, now Patent No. 3,515,546, dated June 2, 1970.  
Divided and this application Mar. 25, 1968, Ser. No.  
715,527

Int. Cl. C21d 1/74

U.S. Cl. 148—159

4 Claims

### ABSTRACT OF THE DISCLOSURE

A method for heat-treating aluminum alloys wherein the completely solidified material is solution and homogenization heat-treated in a vacuum environment at a temperature in the range extending from the alloy solidus temperature to the alloy solid solubility limit temperature a sufficient time to develop improved physical and metallurgical properties upon subsequent cooling and aging.

### CROSS-REFERENCE

This application is a division of application for U.S. Pat. Ser. No. 712,674, filed Mar. 13, 1968 for "Aluminum Alloy Solidification", issued June 2, 1970 as U.S. Pat. No. 3,515,546, and assigned to the assignee of this application.

### SUMMARY OF THE INVENTION

Aluminum alloys having a significant zinc, magnesium, or other strong hydride former content, and particularly if melted, poured, or solidified in an environment containing excessive hydrogen, hydrocarbon, or water vapor constituents, are solution and homogenization heat-treated in accordance with this invention in a vacuum environment at a temperature in the range extending from the alloy solidus temperature to the alloy solid solubility limit temperature a sufficient time. For 7075-type aluminum alloys modified for casting applications, for instance, heat-treatment in a vacuum of  $2 \times 10^{-4}$  mm. Hg at a temperature of  $860^{\circ}$  F.  $\pm 40^{\circ}$  F. for 24 hours per 0.1" of solidified alloy thickness aids substantially in obtaining improved physical and metallurgical properties. Afterwards, the solutioned and homogenized alloy is preferably immediately quenched and subjected to post-heat-treat aging such as on an accelerated basis by heating at from  $250^{\circ}$  F. to  $450^{\circ}$  F. for from 24 hours to 2 hours.

### DETAILED DESCRIPTION

The heat-treating method of this invention has application to the type of aluminum alloy detailed as to composition in the following Table I:

TABLE I

|                                | Modified<br>7075-type | Alloy<br>220 | Experi-<br>mental<br>alloy W |
|--------------------------------|-----------------------|--------------|------------------------------|
| Constituent:                   |                       |              |                              |
| Zinc.....                      | 6.10                  | <0.10        | 4.5                          |
| Magnesium.....                 | 2.31                  | 10.1         | 5.0                          |
| Copper.....                    | 1.18                  | <0.10        | —                            |
| Titanium.....                  | 0.15                  | 0.18         | 0.17                         |
| Beryllium.....                 | 0.11                  | 0.16         | 0.12                         |
| Chromium.....                  | <0.01                 | <0.01        | <0.01                        |
| Manganese.....                 | <0.01                 | <0.01        | <0.01                        |
| Iron.....                      | 0.09                  | 0.05         | 0.06                         |
| Silicon.....                   | 0.09                  | 0.06         | 0.06                         |
| Aluminum.....                  | Balance               | Balance      | Balance                      |
| Total.....                     | 100.00                | 100.00       | 100.00                       |
| Liquidus temperature, ° F..... | 1,175                 | 1,120        | 1,165                        |
| Solidus temperature, ° F.....  | 875                   | 840          | 1,022                        |

Such compositions are stated on a percentage part by weight basis and are characterized as having a significant

## 2

zinc, magnesium, or other strong hydride former content.

The instant invention does not involve melting, pouring, or completely solidifying alloy compositions and such may be accomplished conventionally or even in accordance with the pre-heat treatment method disclosed and claimed in the above-cross-reference application for United States patent, for instance, depending on application requirements. However, significant advantages may be attained if the completely solidified alloy is solution and homogenization heat-treated according to the following method, particularly if alloy melting, pouring, or solidification prior to heat-treatment has been accomplished in an environment having excess hydrogen, hydrocarbons, or water vapor.

The first step in the preferred solution and homogenization heat-treating method involves placing the solidified aluminum alloy having a significant zinc, magnesium, or other strong hydride former content in a furnace chamber that may be sealed and pumped down to a continuous vacuum condition. Solution and homogenization is then accomplished after the chamber pressure is reduced to a vacuum such as  $2 \times 10^{-4}$  mm. Hg. (absolute). The preferred temperature for such heat-treating will vary in relation to the alloy composition. In the case of the modified 7075-type material,  $860^{\circ}$  F.  $\pm 40^{\circ}$  is generally preferred. Alloy 220 can be heat-treated at a temperature in the range of  $800^{\circ}$  F.  $\pm 40^{\circ}$  F.;  $950^{\circ}$  F.  $\pm 40^{\circ}$  F. is considered satisfactory for heat-treating the other alloy detailed as to composition in Table I. Such heat-treating temperatures, in each instance, are in the temperature range from the alloy solidus temperature to the alloy solid solubility limit temperature. For the alloys specified in Table I, 24 hours at temperature per 0.1" of metal thickness is generally satisfactory from the standpoint of time.

Post-heat-treat cooling follows the vacuum solution and homogenization heat-treating step and preferably occurs at cooling rates that are sufficiently high to obtain a non-equilibrium metallurgical structure. It is therefore preferred that the alloys of Table I be immediately quenched from the solution and homogenization heat-treating temperature to ambient temperature in ambient temperature water, equipment permitting. This differs from the normal practice of accomplishing post-heat-treat cooling in heated water such as  $180^{\circ}$  F., for instance and with an intermediate heating following cooling in air.

Afterwards, the quenched alloy may be aged naturally or by conventional accelerated aging steps. In terms of the aluminum alloys of Table I, accelerated aging temperature-time histories in the range of from  $450^{\circ}$  F. for 2 hours to  $250^{\circ}$  F. for 24 hours are adequate. No environmental controlled atmosphere or environmental controlled pressure is required.

A casting alloy having a composition of the type corresponding to the modified 7075-type aluminum alloy set forth in Table I was melted, poured, and directionally solidified in accordance with the pre-heat-treatment method set forth in the description and drawings of the cross-reference application for United States patent. The mold cavity incorporated the external configuration of a missile fin and included a joining riser region positioned above the fin configuration region. A portion of the completed casting was solution and homogenization heat-treated in a  $2 \times 10^{-4}$  mm. Hg continuously pumped vacuum environment at a temperature of approximately  $860^{\circ}$  F. for 48 hours. Since the available heat-treating equipment did not permit quenching directly from temperature, the part was air-cooled after solution and homogenization heat-treating and afterwards heated to  $860^{\circ}$  F. in an air furnace for 2 hours and then water-quenched as specified. Round tensile test bars were machined from coupons

cut from the casting and were found to have the properties set forth in the following Table II.

TABLE II

| Bar Location | Ultimate tensile strength | Yield strength | Percent elongation | RB hardness |
|--------------|---------------------------|----------------|--------------------|-------------|
| Top-----     | 71,200                    | 66,100         | 2.6                | 82.5        |
| Top-----     | 72,000                    | 66,300         | 2.5                | 85.5        |
| Top-----     | 72,700                    | 67,300         | 2.3                | 85          |
| Middle-----  | 72,500                    | 66,800         | 2.7                | 83          |
| Do-----      | 72,200                    | 67,000         | 2.7                | 84.5        |
| Do-----      | 72,400                    | 66,500         | 3.1                | 87          |
| Do-----      | 72,600                    | 66,800         | 2.6                | 85          |
| Bottom-----  | 72,300                    | 66,800         | 2.5                | 83.5        |
| Do-----      | 72,100                    | 66,600         | 2.1                | 83.5        |
| Do-----      | 71,500                    | 65,000         | 2.4                | 84          |

Another portion of the same casting was subjected to 15 a different heat-treatment and then subjected to testing. Specifically, the solidified 7075-type alloy was solution and homogenization heat-treated conventionally in an argon atmosphere just above standard atmospheric pressure at a temperature of 860° F. for 72 hours. The casting 20 portion was air-cooled, reheated to 860° F. for 2 hours in air, water-quenched, and aged as specified (i.e., 24 hours at 250° F.). A coupon from the casting portion so heat-treated, cooled, and aged was found to have a yield tensile strength of 55,300 p.s.i., an ultimate tensile 25 strength of 56,100 p.s.i., and percent elongation of 1.2%.

The completed and heat-treated casting portions were 30 examined radiographically and found to be free of observable defects, particularly as to pin-hole porosity. The improved physical and metallurgical properties first given above are attributed to the invention claimed herein. Vacuum pressure levels are selected with reference to the apparent volatility of alloy constituents at the metal temperature involved and so as to preclude alloying constituent depletion due to processing requirements. More 35 specifically, a vacuum environment of  $1 \times 10^{-5}$  mm. Hg has been determined to be unsatisfactory in at least one instance wherein the aluminum alloy zinc content was undesirably reduced from 5.5% to 0.2%.

Also by way of example, a casting having an aircraft 40 elevator fitting configuration was cast in an alloy whose melt composition (average) consisted of 1.47% copper, 5.62% zinc, 2.61% magnesium, 0.2% titanium, 0.16% beryllium, <0.1% manganese, <0.1% chromium, 0.1% iron, 0.08% silicon, and the balance aluminum, using the 45 pre-heat-treatment melting, pouring, and directional solidification steps disclosed in the cross-reference application for United States patent. After conventional heat-treating in an argon atmosphere at 860° F. for 72 hours followed by quenching and conventional accelerated aging. Coupons cut from the so-processed casting were found to 50

have ultimate tensile strengths from 58,900 p.s.i. to 70,600 p.s.i., elongations from 1.4% to 4.1%, and hardnesses (average) from  $R_B$  78 to  $R_B$  89. One other coupon from the casting was subjected to solution and homogenization heat-treating as specified above in the description of this invention for an additional 23 hours at 860° F. using a vacuum of  $2 \times 10^{-4}$  mm. Hg. After water-quenching and aging at 250° F. for 24 hours, the coupon was found to have an ultimate tensile strength of 92,200 p.s.i., a 3% elongation, and an average hardness of  $R_B$  82.5.

What is claimed is:

1. A method of heat treating a precipitation hardenable aluminum alloy to develop improved physical and metallurgical properties, comprising the steps of:

(a) heating said alloy in a non-heat-treated solidified condition at a temperature in the temperature range from the alloy solidus temperature to the alloy solid solubility limit temperature and in a vacuum environment at a pressure above the pressure of alloying element depletion by vaporization at temperature a sufficient time to dissolve second phase precipitates contained in said alloy and to compositionally homogenize said alloy.

(b) cooling said heated alloy at a rate sufficient to obtain a non-equilibrium metallurgical structure, and

(c) precipitation hardening said heated and cooled alloy by aging to develop improved physical and metallurgical properties therein.

2. The invention defined by claim 1, wherein said heating is continued for approximately 24 hours per 0.1" of alloy thickness.

3. The invention defined by claim 1, wherein said vacuum environment is at a pressure of approximately  $2 \times 10^{-4}$  mm. Hg absolute.

4. The invention defined by claim 3, wherein said heating is continued for approximately 24 hours per 0.1" of alloy thickness.

#### References Cited

##### UNITED STATES PATENTS

|           |         |                |       |           |
|-----------|---------|----------------|-------|-----------|
| 1,996,379 | 4/1935  | Keller         | ----- | 148—16    |
| 2,221,526 | 11/1940 | Sampson        | ----- | 148—159   |
| 2,995,479 | 8/1961  | Cochran et al. | ----- | 148—13.1  |
| 3,084,080 | 4/1963  | Hunter et al.  | ----- | 148—13.1X |

##### OTHER REFERENCES

Chemical Abstracts, vol. 67, 1967, Abstract No. 46505(e).

CHARLES N. LOVELL, Primary Examiner